

3,505,227  
**LUBRICATING OIL COMPOSITIONS CONTAINING  
 BIS-ALKENYL SUCCINIMIDES OF XYLYLENE  
 DIAMINES**

Warren Lowe, El Cerrito, Calif., assignor to Chevron Research Company, San Francisco, Calif., a corporation of Delaware  
 No Drawing. Filed Dec. 18, 1967, Ser. No. 691,225  
 Int. Cl. C10m 1/30, 1/32  
 U.S. Cl. 252—51.5

4 Claims

**ABSTRACT OF THE DISCLOSURE**

Bis-alkenyl succinimidyl alkyl benzenes having from 0 to 4 halogens on the benzene ring find use as lubricating oil detergents. The alkenyl group has from 40 to 125 carbon atoms.

**BACKGROUND OF THE INVENTION**

## Field of the invention

The modern lubricating oil contains detergents and dispersants to prevent the formation of deposits and the depositing of sludge in internal combustion engines. To be an acceptable detergent, not only must the additive have good detergency, but its decomposition products must not enhance the formation of deposits. Moreover, the economics of lubricating oil detergents require that a satisfactory detergent be effective not only under the "hot" conditions of the diesel engine, but the more variable "cold" conditions of the automobile engine.

## Description of the prior art

Ashless detergents comprising the reaction product of a carboxylic acid of relatively high molecular weight with a variety of amines have been reported in U.S. Patent Nos. 3,024,237, 3,275,554, 3,219,666 and 3,172,892. The preferred compositions have been the alkenyl succinic anhydrides of alkylene propylamines, although other amines and amine derivatives have also been disclosed.

**SUMMARY OF THE INVENTION**

Pursuant to this invention, compositions having excellent detergency and detergent capability and being capable of retaining this capability for long periods of time, while being compatible with a wide variety of other lubricating oil additives, are provided, which are bis-alkenyl succinimidyl alkyl benzenes, wherein the alkenyl group is of from about 40 to 125 carbon atoms. The benzene ring may have from 0 to 4 halogen atoms, particularly of atomic No. 17 to 35.

**DESCRIPTION OF THE PREFERRED EMBODIMENTS**

For the most part, the compositions of this invention will have the following formula:



wherein X is halogen of atomic No. 17 to 35 (chlorine or bromine) preferably chlorine, n is an integer of from 0 to 4, preferably 0 to 2 to 4 and A is of the formula:



wherein R is a branched chain oil solubilizing aliphatic group of from 40 to 125 carbon atoms, more usually of from 50 to 100 carbon atoms, and U is alkylene of from 1

to 2 carbon atoms, i.e., methylene and ethylene. The bracket indicates the two positions to which A may be bonded on the benzene ring.

As indicated from the above formula, the alkenyl succinimidyl alkyl groups may be situated meta or para or there may be a mixture of the two. The halogens may be situated at any of the remaining places. The aliphatic hydrocarbyl succinimidyl alkyl groups in being situated meta or para, are separated by at least 3 annular carbon atoms.

10 The aliphatic hydrocarbon radical may be aliphatically saturated or unsaturated, usually having not more than 2 sites of unsaturation, more usually not more than 1 site of unsaturation. There should be at least 1 branch per 4 carbon atoms along a chain and preferably at least 1 branch per 2 carbon atoms along a chain. The branch will ordinarily be a methyl group (1 carbon atom). Illustrative aliphatic hydrocarbyl groups are polyisobutylene, polypropenyl, the copolymer of ethylene and isobutylene, etc. 15 These groups may be readily obtained by polymerizing aliphatic olefins of from 2 to 6 carbon atoms, more usually of from 3 to 4 carbon atoms.

Particularly preferred compositions of this invention have the following formula:



wherein R<sup>1</sup> is a polyolefin of olefins of from 3 to 4 carbon atoms, e.g., polypropylene or polyisobutylene, having from 40 to 125 carbon atoms, preferably 50 to 100 carbon atoms, and n<sup>1</sup> is an integer of from 0 to 4, preferably 0 or 2 to 4. A preferred orientation for the succinimidyl radical is para. Also preferred is a mixture of meta and para having at least 50% meta, usually 50 to 80 mole percent meta.

**PREPARATION OF THE COMPOSITIONS**

The compositions of this invention are readily prepared by combining the desired aliphatic hydrocarbon substituted succinic anhydride of the formula:



wherein R is as defined previously with an amine of the formula:



wherein U, X and n are all as defined previously, either neat or in the presence of a hydrocarbon solvent. Usually, about stoichiometric amounts of materials will be used, a small excess of the succinic anhydride being preferred.

60 The temperature for the reaction will generally be in the range of about 125° C. to 250° C., more usually in the range of about 150° C. to 200° C. The time for the reaction will range from about 30 minutes to 6 hours, the course of the reaction being followed by the evolution of water.

**EXAMPLES**

The following examples are offered by way of illustration and not by way of limitation.

**Example I**

(A) Into a reaction flask was introduced 55 g. of xylylene diamine (70% meta; 30% para) 1,745 g. of a

40 weight percent solution in neutral oil of polyisobutetyl succinic anhydride (polyisobutetyl group of about 1,000 molecular weight) and 150 cc. of benzene. The mixture was heated at reflux, collecting water in a Dean Stark Trap, and the temperature slowly raised to a final temperature of about 170° C. while taking the benzene overhead. A mild vacuum was then applied to the mixture for about one-half hour while maintaining the temperature. The residue was filtered hot and the product isolated.

Analysis (percent).—N=0.60.

Example II

Into a reaction flask was introduced 68.5 g. of 2,3,5,6-tetrachloro-paraxylylene diamine, 1,090 g. of a 40 weight percent solution in neutral oil of polyisobutetyl succinic anhydride (polyisobutetyl of about 1,000 molecular weight) and 300 cc. of benzene. The mixture was heated and stirred at reflux and the water removed as formed. The temperature was slowly raised to 160° C. while taking water and solvent overhead. The temperature was then held for 15 minutes while a mild vacuum was applied to the system. The product weighed 1,151 g. Analysis (percent).—N=0.62.

The compositions of this invention may be used under a wide variety of conditions in internal combustion engines. These compositions, however, find particular use under the hot conditions of diesel engines working under severe conditions of operation.

The compositions of this invention may be formulated with various lubricating fluids (hereinafter referred to as oils) which are either derived from natural or synthetic sources. Oils generally have viscosities of from about 35 to 50,000 Saybolt Universal Seconds (SUS) at 100° F. Among natural hydrocarbonaceous oils are paraffin base, naphthenic base, asphaltic base and mixed base oils. Illustrative of synthetic oils are: hydrocarbon oils such as polymers of various olefins, generally of from 2 to 8 carbon atoms, and alkylated aromatic hydrocarbons; and nonhydrocarbon oils, such as polyalkylene oxides, aromatic ethers, carboxylate esters, phosphate esters, and silicon esters. The preferred media are the hydrocarbonaceous media, both natural and synthetic.

The above oils may be used individually or together whenever miscible or made so by the use of mutual solvents.

When the detergents of this invention are compounded with lubricating oils for use in an engine, the detergents will be present in at least about 0.1 weight percent and usually not more than 20 weight percent, more usually in the range of about 2 to 15 weight percent. The compounds can be prepared as concentrates due to their excellent compatibility with oils. As concentrates, the compounds of this invention will generally range from about 10 to 70 weight percent, more usually from about 20 to 50 weight percent of the total composition.

A preferred aspect in using the compounds of this invention in lubricating oils is to include in the oil from about 1 to 50 mm./kg. of a dihydrocarbyl phosphorodithioate, wherein the hydrocarbyl groups are from about 4 to 36 carbon atoms. Usually, the hydrocarbyl groups will be alkyl or alkaryl groups. The remaining valence of the phosphorodithioate will usually be satisfied by zinc, but polyalkyleneoxy or a third hydrocarbyl group may also be used. (Hydrocarbyl is an organic radical composed solely of carbon and hydrogen which may be aliphatic, alicyclic, aromatic or a combination thereof.)

Other additives may also be included in the oil such as pour point depressants, oiliness agents, antioxidants, rust inhibitors, etc. Usually, the total amount of these additives will range from about 0.1 to 10 weight percent, more usually from about 0.5 to 5 weight percent. The individual additives may vary from about 0.01 to 5 weight percent of the composition.

In order to demonstrate the excellent effectiveness of the compounds of this invention as detergents and dis-

persants in lubricating oils, the compound of Example II was tested in a 1-G Caterpillar test (MIL-L-45199 conditions) for 60 hours. The oil used was a Mid-Continent SAE 30 oil, 12.3 weight percent of this additive was used, and 12 mm./kg. of zinc di(alkylphenyl)phosphorodithioate (the alkyl groups were polypropylene of about 12 to 15 carbon atoms) was included. The following table indicates the results. Also included for comparison are the results for the base oil containing only the phosphorodithioate. The rating of groove deposits is based on a range of 0 to 100, 100 being completely filled grooves. The rating for land deposits is based on a range of 0 to 800, 800 being completely black. The rating for underhead deposits is based on a range of 0 to 10, 10 being completely clean.

TABLE I

| Example | Deposits              |                       |              |  |
|---------|-----------------------|-----------------------|--------------|--|
|         | Groove                | Land                  | Underhead    |  |
| II      | 93-15-5-2<br>19-1-0-0 | 500-800-330<br>70-0-5 | -----<br>9.3 |  |

In order to demonstrate the effectiveness of the compositions of this invention under extremely severe engine conditions, the compositions of Examples I and II were compounded in a Mid-Continent SAE 30 neutral oil at 6.1 and 6.25 weight percent respectively. Also included was 12 mm./kg. of a common oxidation inhibitor; namely, zinc O,O-dialkylphenyl phosphorodithioate (the alkyl groups are from 12 to 14 carbon atoms).

The test used is a particularly severe test which is referred to as the 240 BMEP (brake mean effective pressure) Caterpillar Test. The conditions are for a supercharged caterpillar test wherein the pressure of the supercharged air is 76.5" mercury absolute, the water temperature of the cooling jacket is 200° F., the air temperature is 120° F., the oil temperature of the bearing is 190° F., the sulfur content of the fuel is 0.4 weight percent, the speed of the engine is 1200 r.p.m., and the rate of fuel input is at a rate which provides 6900 B.t.u.'s per minute. The test was carried out for 60 hours and the following table indicates the results. The results are reported as described previously.

TABLE II

| Example | Deposits      |            |           |  |
|---------|---------------|------------|-----------|--|
|         | Groove        | Land       | Underhead |  |
| I       | 34, 1, 0.1, 0 | 30, 0, 0   | 7.5       |  |
| II      | 47, 4, 2, 0.2 | 80, 10, 10 | 8.5       |  |

It is evident from the above results that the compositions of this invention, which are free of basic nitrogen, are readily available from commercially available compounds, easily synthesized to a relatively homogeneous product, and are excellent detergents under the hot conditions of a caterpillar engine, even when carried out under extremely severe conditions.

I claim:

1. A lubricating oil composition having an oil of lubricating viscosity and in an amount sufficient to provide detergency and dispersancy, a material consisting essentially of I or II, or mixtures thereof, wherein I is of the formula:



and II is of the formula:



5

wherein X is halogen of atomic No. 17 to 35, n is an integer of from 2 to 4, and A is of the formula:



5

wherein R is a branched chain oil solubilizing aliphatic group of from 40 to 125 carbon atoms and U is alkylene of from 1 to 2 carbon atoms.

2. A lubricating oil composition according to claim 1 wherein n is from 2 to 4, X is chlorine, and R is of from 50 to 100 carbon atoms.

3. A lubricating oil composition according to claim 2 wherein R is polyisobutylene and U is methylene.

4. A lubricating oil composition having an oil of lubricating viscosity and from 10 to 80 weight percent of a material consisting essentially of I or II, or mixtures thereof,

wherein I is of the formula:



6

and II is of the formula:



wherein X is halogen of atomic No. 17 to 35, n is an integer of from 2 to 4, and A is of the formula:



10

wherein R is a branched chain oil solubilizing aliphatic group of from 40 to 125 carbon atoms and U is alkylene of from 1 to 2 carbon atoms.

#### References Cited

##### UNITED STATES PATENTS

- 20 3,131,150 4/1964 Stuart et al.  
 3,219,666 11/1965 Norman et al.  
 3,306,907 2/1967 McNinch et al.

DANIEL E. WYMAN, Primary Examiner

25 W. J. SHINE, Assistant Examiner